

## UNITED STATES PATENT OFFICE

2,199,125

## ANTIFRICTION METALING OF BEARINGS

Marius Jean-Baptiste Barbarou, Neuilly/Seine,  
FranceNo Drawing. Application February 19, 1938, Se-  
rial No. 191,517. In France February 19, 1937

3 Claims. (Cl. 91—70.3)

The present invention relates to the coating of ferrous metals and alloys with a layer of metal having important frictional characteristics, and in particular alloys with a base principally of tin, 5 with very diverse compounds such as antimony, lead, zinc cadmium or other bodies; these alloys being usually termed "antifriction metal" and the invention has for its object a novel process and means for carrying out the said process in 10 order to obtain perfect adherence of the coating on the metals in question.

It is known that the application of such coatings is to be preceded by a tinning of the metals or alloys to be treated and that the diffusion of 15 the tin in iron is difficult at ordinary temperatures, so that the tinning has only a restricted adhesion on the ferrous alloys. The result is that in the course of working under loads which are generally heavy, a scaling or detachment of 20 the antifriction metal takes place.

The present invention presents a simple means for overcoming these difficulties and is characterised in particular by the introduction of silicon into the ferrous alloys, in the course of an 25 ordinary cementation with ferro-silicon, thus forming at the surface of the alloy a metallic combination of iron and silicon.

Following this the tinning is proceeded with, after certain precautions which will be more explicitly dealt with hereafter, which operation is possible at the usual ordinary temperatures, utilising to this end the natural affinity of silicon for tin, or vice versa. Consequently, this tinning 35 adheres very strongly to the shell, the presence of the silicon enabling it to diffuse regularly to the interior of the metal.

The coating or antifriction metalising proper may be carried out in the ordinary way without special centrifugation.

40 In order that the process which has been described shall have satisfactory results, suitable precautions should be taken in carrying it out.

Presuming that it is desired to provide a bearing with antifriction metal by the process described, the following or a similar procedure 45 should be adopted.

The bearing should be first cemented with ferro-silicon for a period of 5 to 20 hours or

more according to the thickness of the layer desired and at a temperature of approximately 900° C. The cemented bearing will then be immersed in a solution of hydrochloric acid to remove all traces of fatty bodies and then in hydrofluoric acid to dissolve the silica immediately formed by oxidation of the silicon when hot. Any trace of silica would prevent the combination of the silicon and tin, forming an absolute screen.

5 After passing through a solution of zinc chloride, the bearing is tinned at about 350° C. and dipped several times in the chloride of zinc and in the tin bath.

The antifriction metaling should be carried 10 out immediately afterwards.

It is important that these various operations be carried out as quickly as possible to avoid any partial reoxidation of the surfaces.

15 The use of the silicon only serves as intermediary to facilitate the metallic combination of iron and tin which, as is known, is very incomplete at the ordinary tinning temperatures. Any other body than silicon giving the same result is comprised within the scope of the invention.

20 What I claim as my invention is:

1. A process for bonding an antifriction coating to iron and ferrous alloys, comprising the step of subjecting the surface to be treated to a silicon cementation, applying a tin coating to 25 said cemented surface, and thereafter fusing to said tin coating a layer of antifriction metal.

2. In a process of the character described, the steps of subjecting an iron or ferrous alloy surface to a cementation with ferrosilicon at a temperature of 900° C. for a period of from 5 to 20 hours, acid-cleaning the cemented surfaces to remove silica, applying a tin coating to the cleaned surfaces, and thereafter fusing to the 30 tin an antifriction metal layer.

3. A process for bonding an antifriction coating to iron and ferrous alloys, comprising the steps of subjecting the surface to be treated to a silicon cementation, applying zinc chloride to 35 said cemented surface, tinning the cemented surface, and thereafter fusing to said tinned surface a layer of antifriction metal.

40 MARIUS JEAN-BAPTISTE BARBAROU.